

Jan. 17, 1956

M. BACHNER

2,731,046

TOW TARGET

Filed Oct. 1, 1951



INVENTOR.  
Martin Bachner  
BY  
Eug. Frye

Atty's-

1

2,731,046

## TOW TARGET

5

Martin Bachner, Pottstown, Pa., assignor to The Firestone Tire & Rubber Company, Akron, Ohio, a corporation of Ohio

Application October 1, 1951, Serial No. 249,116

10

3 Claims. (Cl. 139—420)

This invention relates to banner tow targets for towing through the air by an airplane or other suitable means, for target practice by gunners in other aircraft or on the ground. Targets of this type present several problems. They must be of a material which has minimum drag and is strong enough to resist tearing or fraying by being towed at high rates of speed, often 300 miles per hour or more. Such targets are usually made of a rectangular piece of fabric attached to a suitable tow line for fastening to the towing means. The fabric is preferably woven from monofilament material in order to avoid unraveling and twisting characteristic of multifilament yarns.

One of the problems encountered in developing tow targets from monofilament yarns resides in the fact that most synthetic monofilaments tend to become brittle at the low temperatures encountered at high altitudes. Many synthetic monofilaments which have excellent strength and flexibility at ordinary air temperatures, 40 to 100° F., become quite brittle, and are easily broken, at temperatures about —40° F., which is typical at high altitudes. Previously tried synthetic materials which have been especially plasticized to make them flexible at low temperatures do not have satisfactory strength at the higher temperatures mentioned, and are often quite flabby at these higher temperatures.

Another problem encountered in the development of the tow targets has been to produce a fabric having high trapezoidal tear resistance. This characteristic is considered necessary for a successful tow target fabric, in order to minimize tears which might result from air-drag and also projectile holes. Many fabrics of high strength filaments have fallen down in this respect, for reasons not clearly understood.

Still another problem encountered in attempts to use synthetic fabrics in tow targets is to prevent deterioration of the targets by action of sunlight and other atmospheric factors. Many synthetic materials exhibit very desirable physical properties when maintained out of sunlight and away from oxidizing conditions, but undergo rapid deterioration when exposed to the sun and air.

It is therefore an object of this invention to provide an improved tow target for use in the air, which successfully solves the problems enumerated above. Specifically, it is an object to produce a banner tow target made of fabric woven from synthetic monofilament material, the fabric possessing satisfactory strength at all temperatures encountered in actual use, having high trapezoidal tear characteristics, remaining flexible at low temperatures as well as at high temperatures, being substantially unaffected by sunlight and air, and resisting tearing when towed through the air at high rates of speed and when perforated by projectiles. It is also a specific object to provide an economical tow target which may be readily manufactured at low cost. An additional object is to produce tow targets capable of detection by radarscope.

The above and further objects will be apparent in the description of the invention which follows, and in the single sheet of drawing, in which:

2

Fig. 1 is a schematic side elevation of a tow target of the invention attached to a towing airplane;

Fig. 2 is a fragmentary view of an open weave square woven fabric for use in the tow target of the invention;

Fig. 3 is a fragmentary view of an open weave leno fabric for use in the tow target of the invention;

Fig. 4 is a perspective view, partly in section, of a foil-coated monofilament of a modified embodiment of the invention; and

Fig. 5 is a perspective view, partly in section, of a metal-coated monofilament of another modified embodiment of the invention.

The objects of the invention are accomplished by fabricating the tow target from a suitable fabric woven of polyethylene monofilament yarn. The polyethylene is suitably unplasticized and may contain no pigments or other compounding ingredients, although suitable pigments may be incorporated if desired.

Although polyethylene has proved to be quite successful in film for food wrapping, and other uses which are satisfied by a relatively low strength, somewhat flabby material, polyethylene fabric has not heretofore been found acceptable in the textile trade. Polyethylene fabric generally possesses a soft and somewhat flabby feel, when compared with such successful textile fabrics as those made of monofilament nylon and saran. Also, polyethylene fabric is somewhat sensitive to the high temperatures regularly encountered in laundering and pressing operations, since polyethylene is thermoplastic, even though it is crystalline and orientable.

In spite of these apparent drawbacks it has been found in accordance with the present invention that open weave fabrics, such as those shown in Figs. 2 and 3, of polyethylene monofilaments exhibit high trapezoidal tear characteristics, even though the tensile strength of the monofilament yarn is only a fraction of the tensile strength of nylon or saran yarns. It has also been discovered that such polyethylene fabric retains these desirable tear-resistant characteristics over an extremely wide range of temperatures, from below —100° F. to more than 100° F., even though the polyethylene filament contains no added plasticizer. Additionally, it has been proven by actual tests that such polyethylene fabric is quite stable in the presence of sunlight and air, and does not deteriorate rapidly as do similar fabrics of other synthetic monofilaments.

Polyethylene may be extruded in known manner to produce a finished filament 10 having a diameter of approximately 0.010 to 0.050 inch, preferably in the range of 0.019 to 0.023 inch. The filament may be oriented, and may also be given a supplemental heat treatment while under some tension in order to reduce shrinkage, if desired.

The fabric may be manufactured in a variety of open weaves, the two weaves shown in Figs. 2 and 3 being merely illustrative. The locked leno weave shown in Fig. 3 possesses some mechanical advantages over the simple cross woven fabric of Fig. 2, and is a preferred weave. The tow target fabric should be produced with an open weave in order to keep down the weight of the target. The fabric is woven to weigh less than 10 ounces per square yard and preferably in the range of 5 to 7.5 ounces per square yard. The preferred weave is identified as a three-end leno repeating on six picks, which is illustrated in Fig. 3, the warp filaments being identified as 10a, 10c and the fill or weft filaments as 10b, 10b. A suitable fabric produced from filament of 0.020 inch diameter has not less than 12 warp ends per inch and not less than 11 picks per inch in the filling direction. The fabric is preferably selvaged, a selvage of ½ to 1 inch being satisfactory. Such fabric has been found to possess warp and filling breaking strengths of more than 35 pounds

per inch, and elongation of over 30% in the warp and over 25% in the filling.

A target is constructed of polyethylene fabric as described, suitably in the form of a banner approximately 6 feet wide and 30 feet long, designated 11 in Fig. 1. The banner is attached at one end to a harness 12 connected to a tow line 13 for attaching to an airplane 14 or other suitable towing means.

One example of polyethylene monofilament fabric suitable for manufacture of the tow target was an off balance 10 square woven fabric possessing a fabric thickness of approximately 0.020 inch. The fabric possessed the following physical properties:

Tensile strength (1 inch grab method):

|        |      |     |
|--------|------|-----|
| Warp   | lbs. | 118 |
| Filler | lbs. | 74  |

Elongation:

|        |         |    |
|--------|---------|----|
| Warp   | percent | 39 |
| Filler | do      | 65 |

Tear (trapezoid method):

|        |      |    |
|--------|------|----|
| Warp   | lbs. | 86 |
| Filler | lbs. | 48 |

Cold temperature test at -123° F. No cracking

The fabric of the leno weave shown in Fig. 3 was prepared from monofilament polyethylene yarn of approximately 0.020" diameter. This fabric had the following properties:

Tensile strength:

|        |      |      |
|--------|------|------|
| Warp   | lbs. | 53.9 |
| Filler | lbs. | 52.7 |

Elongation:

|        |         |      |
|--------|---------|------|
| Warp   | percent | 41.9 |
| Filler | do      | 45.6 |

Tear (trapezoid method):

|        |      |      |
|--------|------|------|
| Warp   | lbs. | 33.5 |
| Filler | lbs. | 44.3 |

Weight oz. per sq. yd. 2.67

A banner target was prepared from this leno fabric 40 and was flown 30 minutes at 25,000 feet and -20° C., and then an additional 30 minutes at -10° C., without showing any appreciable wear.

A similar target in accordance with the invention was flown a total of 17 missions, total flight time 15 hours, 45 190 miles per hour average speed, at altitudes of 7,000 to 20,000 feet. At the end of this time the tow target had 640 projectile holes but was still considered satisfactory for further use.

Although unpigmented polyethylene filament has been 50 proved to be quite satisfactory in tow targets, it is contemplated that other polyethylene compositions may be used in the invention. For example, carbon black may be incorporated in polyethylene to produce a black filament possessing greater resistance to sunlight aging. Also, conventional organic chemical light and heat stabilizers may be incorporated in polyethylene prior to extruding in filament form. Other colors than black may be incorporated in the polyethylene prior to extrusion, in order to mark the tow target with a distinctive color, or to provide 55 60

colored filament for weaving a desired design into the fabric to be used in manufacturing tow targets. Fluorescent pigments may be incorporated into or onto the filaments or a portion of the filaments of the target to increase its visibility.

By providing polyethylene monofilament with a covering or coating of metal a tow target is produced therefrom which reflects radar waves. This type of target may be used at night or through clouds to provide gunnery practice for an aircraft or ground gunner equipped with a suitable radarscope or similar device. As is shown in Fig. 4, a polyethylene monofilament 15 is covered (or partially covered, if desired) with a spiral wrapping of metal foil 16, aluminum foil being found satisfactory. 15 A tow target produced from fabric woven partially or completely of such foil-wrapped filament is readily visible in a radarscope.

Another modified filament for use in the fabrication of a tow target for radar gunnery practice is shown in 20 Fig. 5. A polyethylene filament 17 is partially or completely covered with a thin layer 18 of metal, as by the "vacuum vapor deposit" technique. Thus, filament is placed in a high vacuum in which a metal (such as aluminum) is vaporized by means of a high frequency electric discharge, and the vaporized metal is allowed to deposit on and adhere to the surface of the filament.

What is claimed is:

1. An aircraft tow target comprising essentially a sheet of an open weave fabric woven of monofilament polyethylene yarn, the diameter of filament being in the range of 0.010 to 0.050 inch, the weight of the fabric being less than 10 ounces per square yard, the breaking strength of the fabric being greater than 35 pounds per inch in both warp and filling, a substantial portion of the yarn carrying a thin coating of metal on the surface thereof.

2. A tow target as in claim 1, in which a substantial portion of the yarn is wrapped in thin aluminum foil.

3. A tow target as in claim 1, in which a substantial portion of the yarn surface comprises a thin adhered layer of metal.

References Cited in the file of this patent

UNITED STATES PATENTS

- |           |               |                |
|-----------|---------------|----------------|
| 1,730,263 | Brooks        | Oct. 1, 1929   |
| 2,210,774 | Perrin et al. | Aug. 6, 1940   |
| 2,238,875 | Manson        | Apr. 15, 1941  |
| 2,357,851 | Scheyer       | Sept. 12, 1944 |
| 2,458,243 | Biddle        | Jan. 4, 1949   |
| 2,511,644 | Liss          | June 13, 1950  |
| 2,523,738 | Trimbach      | Sept. 26, 1950 |

FOREIGN PATENTS

- |       |               |         |
|-------|---------------|---------|
| 4,389 | Great Britain | of 1888 |
|-------|---------------|---------|

OTHER REFERENCES

"The New Fibers," Sherman and Sherman, D. Van Nostrand Co., Inc., N. Y. C. Copyright 1946, pp. 131-141.